

# UNITED STATES PATENT OFFICE.

HARRY P. BASSETT, OF CYNTHIANA, KENTUCKY.

## PROCESS OF BLEACHING COTTON.

1,402,040.

Specification of Letters Patent.

Patented Jan. 3, 1922.

No Drawing.

Application filed April 19, 1920. Serial No. 375,147.

To all whom it may concern:

Be it known that I, HARRY P. BASSETT, a citizen of the United States, residing at Cynthiana, in the county of Harrison and State of Kentucky, have invented certain new and useful Improvements in Processes of Bleaching Cotton, of which the following is a specification.

This invention relates to processes of 10 bleaching cotton and comprises a method of treating cotton fiber wherein the material is treated with a weak acid solution of a definite predetermined strength to hydrolyze the gummy constituents present as impurities 15 in the raw material, washing the material to remove any soluble bodies formed in the hydrolysis, treating with a weak solution of alkali of a definite predetermined strength to form salts of the organic acids formed in 20 the hydrolysis, washing to remove the salts and then treating with a bleaching agent; all as more fully hereinafter set forth and as claimed.

In the production of fibrous material from 25 cotton, it is customary to treat the raw material with a strong solution of an alkali to hydrolyze the typical waxes and gums present as impurities, and which must be removed to produce a good fiber. I have found 30 that this method does not completely remove the impurities from the fiber. The hydrolysis with a strong alkaline solution does not produce entirely soluble salts which may be readily removed from the fiber by 35 washing. It has, therefore, been necessary to employ a relatively large amount of bleaching material to bleach the impurities present which are not removed by the hydrolysis. A further disadvantage of this 40 method resides in the fact that the impurities are present in the finished material and the fiber is inferior in quality.

A further disadvantage of the present 45 methods of treating cotton fibers resides in the fact that there is a tendency of the alkali and the bleaching material to react upon the cellulose, changing the chemical composition and forming oxy-cellulose and similar bodies. This injures the fibrous structure and makes 50 it unsuitable for many uses, such as, for instance, the manufacture of nitro-cellulose and cellulose acetate, etc.

In the present process, I have found that 55 a much better material may be produced at a relatively lower cost if the material is first

hydrolyzed with a weak acid solution of approximately one per cent strength by weight, or less. After the hydrolysis, the material is treated with a weak solution of an alkali of approximately one per cent strength by weight, or less, which forms salts of the organic acids with the hydrolyzed waxes and resins present in the raw material. This treatment with the weak acid solution and the weak solution of an alkali removes all 60 impurities from the cotton fiber, the salts of the organic acids produced by the alkali being soluble and being washed out in the treatment, and being further washed with water to entirely remove the salts. The 65 fibrous material is then ready for the bleaching step and a relatively small amount of the bleach may be used and a finished material obtained free from any coloring or 70 impurities.

The weak alkaline solution used and the 75 relatively small amount of bleach employed removes the possibility of reaction by the alkaline solution or the bleach and the cellulose bodies present in the cotton fiber and thus eliminates the possibility of forming 80 oxy-cellulose and similar bodies, which are detrimental in many uses in which the finished cellulose is employed.

As stated, when the hydrolysis is performed with an alkali, the compounds produced are not all freely soluble in water and the result is that some of the impurities are not removed by the subsequent washing step. Under such conditions, it is necessary to employ a large amount of bleaching material and this is a disadvantage, as the bleaching 90 material itself has a tendency to react upon the cellulose bodies of the fiber and produce oxy-cellulose and similar bodies. In addition, it has been found impossible to completely remove all color from some fibrous 95 materials by the bleaching operation, even when a very strong bleaching solution is employed.

In the present process, the cotton fiber is so treated that the original structure is not injuriously affected and the chemical composition of the cellulose bodies is unchanged, but practically all impurities are removed. 105 When the material is submitted to the bleaching step, only a very small amount of bleach is necessary to remove all color from the fibrous material and produce a practically pure cellulose fiber.

In the present invention, the raw cotton fibers are first treated with the weak acid solution. Any acid which is capable of furnishing a hydrogen ion in the hydrolysis of the typical waxes and resins present as impurities in the raw material may be employed. For commercial purposes, I have found that the mineral acids, such as sulfuric acid and hydrochloric acid are best adapted for the performance of the process, but the invention is in no way limited to the use of either of these acids, or to the use of a mineral acid. The relative cheapness of the mineral acids such as sulfuric acid and hydrochloric acid and their greater efficiency in furnishing the hydrogen ion for hydrolysis makes them preferable in the practice of the process from a commercial standpoint.

The acid treatment removes the sugar originally present in the typical waxes and resins, and may wash out some of the more soluble organic acids formed by hydrolysis. The material is then submitted to washing to remove any other soluble bodies present before treatment with the alkali. It is then treated with a weak solution of an alkali, such as any basic compound of an alkali or alkaline earth metal which will combine with the organic acids to form soluble salts of the organic acids. I have found that sodium and potassium compounds, such as sodium or potassium carbonate, caustic soda, or caustic potash, are well suited for this operation, but the invention is not limited to the use of any of the materials mentioned.

After the treatment with the alkali, the impurities present are all in the form of soluble salts of the organic acids and they may be readily removed by washing. This operation is best performed with hot water, the material being washed in any of the usual methods until all, or practically all, of the impurities are removed. The material is then ready for the bleaching operation, and the cellulose bodies forming the fiber are present in a chemically unchanged condition due to the relative weakness of the acid and alkaline solutions used, but in a physical condition particularly adapted to respond readily to the action of the bleaching agent. The impurities are practically all removed by the treatment with the acid and alkaline solutions and the subsequent washing steps, and a very small amount of a bleaching agent may be used. Any of the well known bleaching agents may be employed and I have obtained a practically white fiber by bleaching the material in the usual manner with a solution of calcium hypochlorite, containing a fraction of one per cent of the bleaching agent.

While I prefer to employ solutions of acid and alkali of one per cent strength or less, I have found that satisfactory results may

be obtained by employing solutions of from five-tenths to one and one-half per cent strength. In the case of the acid, I have obtained commercially satisfactory results by using a strength of one-fourth of one per cent, and in the case of the solution of alkali, I have obtained commercially satisfactory results from the use of a solution having a strength as high as two and one-half per cent.

I am aware that a weak solution of acid has been used to hydrolyze typical waxes and loosen the fiber of flax, straw, and the like from the shive, and that a weak solution of acid has been used to loosen or separate the fiber of flax and like material from the shive, and that the combined use of both steps has been proposed, as set forth in Letters Patent No. 1,046,536, granted to me December 16, 1912.

It is, however, well understood by chemists familiar with flax and like stalks, that their physical composition is rugged and that their chemical make-up differs substantially from that of cotton, particularly in respect of the binding agents of the fibers.

I am also aware that it has been proposed to treat cotton fibers with a weak solution of an alkali followed by a weak solution of an acid, but the advantages of the present process cannot be obtained by such treatment; nor by treating cotton fibers with a strong acid solution followed by the use of either a weak or a strong solution of an alkali; nor by the treatment with a strong acid solution after a preliminary treatment with a weak acid solution.

Having thus described my invention, I claim:

1. The process of bleaching cotton fibers which comprises hydrolyzing the typical gums and resins present in the fibers with an acid solution of not in excess of substantially one and one-half per cent strength to form soluble sugars and organic acids, washing to remove the sugars and the soluble organic acids, treating with an alkaline solution of not in excess of substantially two and one-half per cent strength to form salts of the organic acids, washing to remove the salts formed, and bleaching.

2. The process of bleaching cotton fibers which comprises hydrolyzing the typical gums and resins present in the fibers with a solution of mineral acid of substantially less than one per cent strength, washing to remove the sugars and the soluble organic acids, treating with an alkaline solution of not in excess of approximately two and one-half per cent strength, to form salts of the organic acids, washing to remove the salts formed, and bleaching.

3. The process of bleaching cotton fibers which comprises hydrolyzing the typical gums and resins present in the fibers with an

acid solution of not in excess of substantially one per cent strength, washing to remove the sugars and the soluble organic salts, treating with an alkaline solution of not in excess of substantially one per cent strength to form salts of the organic acids, washing to remove the salts formed, and bleaching.

4. The process of bleaching cotton fibers which comprises hydrolyzing the typical gums and resins present in the fibers with an acid solution of substantially less than one per cent strength, washing to remove the sugars and the soluble organic acids, treating with an alkaline solution of not in excess of one per cent strength to form salts of the organic acids, washing to remove the salts formed, and bleaching.

5. The process of bleaching cotton fibers which comprises hydrolyzing the typical gums and resins present in the fibers with a solution of sulfuric acid of not in excess of approximately one per cent strength, wash-

ing to remove the sugars and the soluble organic acids, treating with a solution of caustic soda of not in excess of approximately one per cent strength to form salts of the organic acids, washing to remove the salts formed, and bleaching.

6. The process of bleaching cotton fibers which comprises hydrolyzing the typical gums and resins present in the fibers with an acid solution of substantially less than one per cent strength, washing to remove the sugars and the soluble organic acids, treating with a solution of caustic soda of not in excess of one per cent strength to form salts of the organic acids, washing to remove the salts formed, and bleaching.

In testimony whereof I affix my signature in presence of a witness.

HARRY P. BASSETT.

Witness:

MARY F. LYONS.